

1,597,000

Patented Aug. 24, 1926.

# UNITED STATES PATENT OFFICE.

BY RAMJI D. SAKLATWALLA, OF CRAFTON, PENNSYLVANIA.

## REFINING SILICON-CONTAINING IRON-CHROMIUM ALLOYS.

No Drawing.

Application filed March 11, 1922. Serial No. 543,085.

The present invention relates to refining silicon-containing iron-chromium alloys, and particularly to a process for refining such alloys in which the silicon is oxidizable without substantial oxidation of the chromium. The invention is particularly applicable to the refining of high silicon ferro-chromium and will be described with particular reference to it, it being understood however that the process may be used for the refining of other silicon-containing iron-chromium alloys, such for example as chrome steels or irons. The ferro-chromium alloy, which is high in silicon, is smelted with an oxidizing agent which oxidizes the silicon without substantially oxidizing the chromium. As such an oxidizing agent, I have used calcium carbonate. The calcium carbonate upon heating yields carbon dioxide which, in turn, yields a part of its oxygen to oxidize the silicon. The calcium carbonate is preferably mixed with calcium oxide which apparently serves as a diluent and which, together with the calcium oxide produced from the calcium carbonate by the liberation of its carbon dioxide, combines with the silica formed by the oxidation of the silicon. It is found that when the high silicon ferro-chromium is smelted with the calcium carbonate and calcium oxide, the silicon can be oxidized without any appreciable oxidation of the chromium. The mixture of calcium carbonate and calcium oxide may be used alone, but it is found that the silicon content can be reduced to a greater extent, say under  $\frac{1}{10}$  of one per cent for special purposes, by the addition of a small quantity of potassium or sodium nitrate, or chrome or iron ore, or a mixture of them, to the calcium carbonate and calcium oxide mixture. The activity of the oxidizing reaction can be controlled by regulating the current density and voltage in the furnace. Increasing the temperature by increasing the current density or voltage, increases the activity of the reaction. I have found that it is possible thus to oxidize the silicon content without any appreciable sacrifice of the chromium content.

Slight additions of fluorspar to the oxidizing mixture are in some cases desirable to facilitate the refining.

Typical examples of the oxidizing mixture are:

55 200 lbs. calcium carbonate, 300 lbs. cal-

cium oxide, 50 lbs. chrome ore, 50 lbs. iron ore, 50 lbs. fluorspar, or  
200 lbs. calcium carbonate, 300 lbs. calcium oxide, 100 lbs. sodium nitrate, or  
200 lbs. calcium carbonate, 300 lbs. calcium oxide, 50 lbs. chrome ore, 50 lbs. sodium nitrate, 50 lbs. fluorspar.

As an example of the composition of the refined alloy, may be cited:

Alloy previous to refining:

|    | Per cent. |
|----|-----------|
| Cr | 39.46     |
| Si | 34.4      |
| C  | 0.22      |

Alloy after refining:

|    | Per cent. |
|----|-----------|
| Cr | 65.80     |
| Si | 0.03      |
| C  | 0.16      |

Another example is as follows:

Alloy previous to refining:

|    | Per cent. |
|----|-----------|
| Cr | 15.61     |
| Si | 26.50     |
| C  | 0.59      |

Alloy after refining:

|    | Per cent. |
|----|-----------|
| Cr | 63.70     |
| Si | 2.03      |
| C  | 0.34      |

The oxidizing mixture is added to the high silicon ferro-chromium, which is in the molten state. The oxidizing mixture is preferably added in successive installments until an analysis of a sample shows that the silicon content of the alloy has been reduced to the desired percentage.

While I have specifically described the preferred way of carrying out my process, it is to be understood that the invention is not limited to the described details, but may be otherwise embodied within the scope of the following claims.

I claim:

1. The process of refining silicon-containing iron-chromium alloys, which consists in smelting the alloy with a mixture containing calcium carbonate, calcium oxide and a small amount of a nitrate, substantially as described.

2. The process of refining silicon-containing iron-chromium alloys, which consists in smelting the alloy with a mixture containing calcium carbonate, calcium oxide, and

100

110

a small quantity of a nitrate and chrome or iron ore, substantially as described.

3. The process of refining high silicon iron-chromium alloys, which comprises 5 treating the alloy in the molten state with calcium oxide and calcium carbonate in an amount sufficient to act as an oxidizing agent, substantially as described.

4. The process of refining high silicon 10 iron-chromium alloys, which comprises treating the alloy in the molten state with calcium oxide, chromium or iron oxide, and calcium carbonate in an amount sufficient to act as an oxidizing agent, substantially as 15 described.

5. The process of refining high silicon iron-chromium alloys, which comprises treating the alloy in the molten state with a carbonate decomposable at furnace temperatures in an amount sufficient to act as an 20 oxidizing agent, substantially as described.

6. The process of refining high silicon iron-chromium alloys, which comprises subjecting the alloy in a molten state to the 25 oxidizing action of calcium carbonate, substantially as described.

In testimony whereof I have hereunto set my hand.

BY RAMJI D. SAKLATWALLA.